

## UNITED STATES PATENT OFFICE.

WESLEY J. BECK AND JAMES A. AUPPERLE, OF MIDDLETOWN, OHIO, ASSIGNEES TO THE AMERICAN ROLLING MILL COMPANY, OF MIDDLETOWN, OHIO, A CORPORATION OF OHIO.

## IRON ALLOY.

No Drawing.

Application filed July 26, 1919. Serial No. 313,611.

To all whom it may concern:

Be it known that we, WESLEY J. BECK and JAMES A. AUPPERLE, citizens of the United States, and residents of Middletown, in the county of Butler and State of Ohio, have invented a certain new and useful Iron Alloy, of which the following is a full, clear, and exact description.

Our invention relates to iron alloys which have as their object the resistance to the effects of alternate heating and cooling in the presence of air. If any steels, but very special alloys, are subjected to a high temperature, say from a dark red heat and upward to melting point, and permitted at the same time to come in contact with the air, they will form a crust or scale on their surface due to oxidation. This scale is heavy and on account of having a different co-efficient of expansion from the metal will become detached therefrom upon cooling so as to fall off or become dislodged, leaving the alloy reduced in thickness. Ordinary sheet iron or sheet steel therefore deteriorates very rapidly when subjected to alternate heating and cooling, especially where high temperatures are employed, such as used for certain distillation apparatus, stoves, annealing boxes, and many of the various uses in the arts employing high temperatures.

It is our object to provide a new mild steel or workable steel for the purposes of exposure under oxidizing conditions at high temperatures which will not be subjected to the rapid oxidation and deterioration above referred to, and we have accomplished our object by the use of silicon together with other elements or as substantially the sole alloying element with iron.

In manufacturing our alloy it can be produced by the acid or basic Bessemer, open-hearth, electric furnace, or crucible processes. The refining of the metal is preferably carried to the same degree as is ordinarily practiced in the production of mild steel. As is the usual practice in the manufacture of ordinary steel, enough manganese can be added to the metal either in the furnace or in the ladle to produce the de-

sired working qualities. The silicon is preferably added as a ladle charge, otherwise the silicon, especially where oxidizing conditions have prevailed, would have a tendency to react with the slag. The amount of silicon in the final metal may vary five-tenths of one percent, which will give some results, up to whatever percent will admit of working the alloy into the desired shape and produce the desired rolling and forging qualities and ductility, or as expressed in general terms "workability". We prefer to employ from two percent to four and one-half percent, although with other metals in the alloy and special treatment the amount may be increased above this. These percents refer to the amount of silicon in the finished product, and there should be at least five-tenths percent to have a substantial amount of the silicon.

In practice, the new property imparted to steel by the addition of silicon does not give its striking results until somewhere around two percent has been reached, and the five-tenths percent is given as the beginning, so far as we have been able to determine of the evidence of the new effect.

We have been able to take two samples of silicon steel, one containing about two and four-tenths per cent of silicon, and the other about four per cent silicon, which we subjected in an electric furnace to a temperature of 900° C., with the current of air blowing over them. The samples were removed from the furnace periodically, thoroughly cooled and pounded with a hammer in an attempt to dislodge the protective coating. After each period of heating, cooling, and pounding the samples were weighed.

After a hundred hours of this treatment, the samples seemed to have changed in no respect from their condition at the beginning of the test, and for the first sixty hours they gained slightly in weight even though subjected to hammering; this being due to the oxidized coating produced from heating the metal in the presence of air, and after one hundred hours there was but a very slight loss in weight. A sample of ordinary

sheet steel, however, of like size and gauge to the samples mentioned and similarly treated, went to pieces at the end of sixty hours.

- 5 So far as physical appearance was concerned, the result of the first heat treatment was to form an oxidized coating on the samples which was hard or cementlike, and of a smooth or velvetlike finish. This finish 10 could not be marred by the rough treatment administered, and remained, to all intents and purposes, entirely unaltered during the entire treatment.

Thus it may be seen from this experiment, 15 which is only briefly referred to, in order to illustrate the properties which we have discovered in silicon steel, that we have made a discovery of very great value in the art, and have opened up a new use to mild and 20 inexpensive steels, which has hitherto been considered impractical. Furthermore a simple heat treatment of the alloy referred to results in forming a flexible coating on the surface of the metal, which is more 25 adherent and fully as attractive in appearance as the coatings formed at high temperatures with the use of gas and superheated steam produced by other processes known in the art.

30 We are aware that others have employed mild silicon steels for various purposes, but so far as we are advised, the new property now fully noted has never before been known, and such silicon steels have never before been employed in the arts for subject 35 tion to the oxidation under conditions of high heat.

By high heat, we mean such a heat as 40 would result in the forming of an oxidized scale on ordinary sheet iron and steel if subjected to the air. Such a heat is to be found as a condition in fuel burning appliances and accessories used with them, as a usual thing, and thus it can be readily observed 45 that the new property discovered of mild silicon steels, and the new use for said steels, under which this property becomes of value, are of great importance, and that the new use occupies a large field which is quite distinct from other uses of iron and its alloys.

50 As a typical analysis of the alloy which will give excellent results in resisting the action of high temperatures under oxidizing conditions, we give the following:

Per cent.

|            |       |
|------------|-------|
| Silicon    | 2.400 |
| Carbon     | .120  |
| Manganese  | .250  |
| Sulphur    | .040  |
| Phosphorus | .025  |
| Nitrogen   | .002  |
| Oxygen     | .005  |

and when using higher silicon another analysis which has proven satisfactory is—

|           | Per cent. |
|-----------|-----------|
| Silicon   | 4.000     |
| Carbon    | .080      |
| Manganese | .200      |
| Sulphur   | .035      |
| Nitrogen  | .003      |
| Oxygen    | .005      |

These analyses are given for examples merely of a means for gaining the advantage of our invention, and not as limitations 75 of the claims that follow except where their wording directly incorporates such details.

The working of our alloy, together with the heat treatments are the same as used 80 and known to the art for providing the desired shapes and characteristics of ductility, malleability, or stiffness in the finished product.

By the words "iron alloys" in the appended claims, we do not intend to limit ourselves to alloys containing iron and silicon only, as the alloy might contain nickel, copper, cobalt, manganese, carbon, arsenic, or any other of the usual alloying constituents 90 together or separately.

For example copper around .25% could be present in either of the above formulæ, and has been employed by us.

Having thus described our invention, what 95 we claim as new and desire to secure by Letters Patent, is:

1. A workable iron alloy which has the characteristic of resisting destructive corrosion at high temperatures under oxidizing conditions and is fabricated into forms for use under exposure to such conditions containing silicon in proportions ranging upward from substantially two per cent to percentage not so high as to render it unworkable and containing more silicon than 105 any other alloying metal.

2. A workable iron alloy which has the characteristic of resisting destructive corrosion at high temperatures under oxidizing conditions and is fabricated into forms for use under exposure to such conditions containing silicon in proportions sufficient to bring about formation on the surface of the metal of a permanent protective coating 115 of cementitious nature and containing more silicon than any other alloying metal.

3. A workable iron alloy which has the characteristic of resisting destructive corrosion at high temperatures under oxidizing conditions and is fabricated into forms for use under exposure to such conditions containing silicon in proportions sufficient to bring about formation on the surface of the metal of a permanent protective coating of cementitious nature, said silicon content running from around two per cent up to around four and one half per cent and containing more silicon than any other alloying metal.

WESLEY J. BECK.  
JAMES A. AUPPERLE.